

1

2,927,012

## FUEL OIL COMPOSITION

Robert J. Hartle, Gibsonia, Pa., assignor to Gulf Research & Development Company, Pittsburgh, Pa., a corporation of Delaware

No Drawing. Application December 18, 1957  
Serial No. 703,498

7 Claims. (Cl. 44—57)

This invention relates to hydrocarbon fuel oils having improved ignition characteristics. More particularly, the invention relates to hydrocarbon fuel oils containing addition agents that are adapted to enhance the ignition and combustion characteristics of such oils.

Hydrocarbon distillates and residual-containing oils having distillation characteristics, viscosities, carbon residues and other properties rendering them otherwise suitable for use as fuels for compression ignition or diesel engines, or other atomizing or vaporizing type burners, frequently have ignition characteristics that render them unsuitable or only poorly suitable for such use. Fuels that have poor ignition characteristics, that is, relatively high spontaneous ignition temperatures, will exhibit an unduly large ignition lag between the time the fuel is injected in the combustion zone and the time when the fuel ignites. In diesel engines, for example, a large ignition lag will result in the combustion of the fuel and the development of pressure over the improper portion of the crank angle period and piston stroke, and this will be accompanied by knocking, rough engine operation, incomplete combustion in the combustion zone, power loss, etc. The ignition quality of diesel fuels is normally expressed in terms of cetane numbers. The cetane number of a given fuel represents the percent proportion of cetane, a fast-burning  $C_{16}$  paraffinic constituent, in  $\alpha$ -methylnaphthalene, a slow burning aromatic material, that will match the performance of the given fuel at the same compression ratio in a standard test engine.

The present invention relates to hydrocarbon fuel oil compositions that possess enhanced ignition quality and other performance characteristics, and which are therefore better adapted for use in diesel engines and other atomizing or vaporizing type burners. I have found that such improved hydrocarbon fuel oil compositions can be obtained by incorporating in the oils a small amount of an aldehyde or ketone cyanohydrin nitrate derived from an aldehyde or ketone having as one substituent a hydrocarbon radical that contains 1 to 18 carbon atoms, and as the other a radical of the same class or hydrogen, whether or not the substituents are separate radicals or different portions of the same radical. The radicals referred to can be saturated or unsaturated, straight or branched chain, cycloaliphatic, aromatic, or heterocyclic. Examples of such radicals include alkyl radicals, such as methyl, n-undecyl, 1-ethylpentyl and n-heptadecyl, alkenyl or alkadienyl radicals such as n-heptadecenyl and n-heptadecadienyl, cycloalkyl radicals such as cyclohexyl and cyclopentyl, aryl radicals such as phenyl and naphthyl, alkaryl radicals such as cresyl and tolyl, aralkyl radicals such as benzyl, and heterocyclic radicals such as furyl. The radicals can be unsubstituted as indicated, or they can be substituted with substituents such as halogen, alkoxy, nitro or the like, that do not adversely affect the oil-solubility or combustion characteristics of the oil or the stability of the resulting cyanohydrin nitrate. The cyano-

2

hydrin nitrates derived from alkyl substituted aldehydes or ketones, particularly those whose alkyl substituents contain 1 to 12 carbon atoms, are especially valuable, acetone cyanohydrin nitrate and 2-ethylhexaldehyde cyanohydrin nitrate being preferred members of the class.

The exact mechanism by which the cyanohydrin nitrates disclosed herein function to improve the ignition characteristics of the fuel oils has not been definitely established. It might appear that these materials function by rapid decomposition at a lower temperature than the spontaneous ignition temperature of the fuel oil, the heat evolved during such rapid decomposition functioning to ignite the fuel oil at a time prior to that at which the spontaneous ignition temperature would be reached. The decomposition of the cyanohydrin nitrates may also promote decomposition of the fuel oil components into materials that are more easily oxidizable and which therefore possess relatively low spontaneous ignition temperatures.

The cyanohydrin nitrates disclosed herein are employed in hydrocarbon fuel oils in a proportion such as to improve the ignition quality of the oil. Such proportion will vary somewhat according to the nature of the fuel oil and on a weight basis according to the nature of the individual cyanohydrin nitrate. Normally, a noticeable improvement in the ignition quality of a fuel oil will be obtained by incorporating therein as little as 0.05 weight percent of the cyanohydrin nitrates disclosed herein, and the use of 0.1 weight percent to 2.0 weight percent will result in a marked improvement. The improvement in ignition quality per unit weight increment of the ketone cyanohydrin nitrates whose use is included by this invention gradually declines somewhat at proportions in the range of about 0.5 to 1.0 weight percent. The rate of decline in improvement per unit increment is greater at proportions in excess of 1.0 weight percent, so that little additional improvement with respect to ignition quality is obtained by the use of proportions in excess of 2.0 percent by weight. The aldehyde cyanohydrin nitrates whose use is included by this invention differ from the ketone cyanohydrin nitrates in that the improvement in ignition quality obtained per unit weight increment ordinarily does not begin to decline at proportions below 1.0 percent by weight. Although the ketone cyanohydrin nitrates are more effective on a weight basis when used in relatively small proportions, it appears that the aldehyde cyanohydrin nitrates produce a greater improvement in ignition quality on a molar basis.

The aldehyde and ketone cyanohydrin nitrates whose use is included by this invention can be prepared in any convenient manner. For example, they can be prepared by esterification of the appropriate cyanohydrin under conditions conventionally employed in esterifying an alcohol with nitric acid, preferably with the use of a molar excess of nitric acid of 70 to 100 percent strength, for example, white fuming nitric acid. In order to avoid oxidation and decomposition of the cyanohydrin nitrates, the reaction temperature is maintained below ambient room temperature (25° C.), preferably below about 15° C., but above the freezing point of the mixture. For example, excellent results are obtained at temperatures in the range of about -5° to 10° C. It is preferred that water of esterification be removed from the reaction by the use of a desiccant, that is, by hydration of an inert material having an affinity for water, which material can also be a solvent for the reactants. An example of a suitable desiccant, or hydratable material, having solvent characteristics is acetic anhydride. Other desiccants include anhydrous sodium sulfate and calcium chloride. The hydratable material is desirably employed in a proportion sufficient to absorb the theoretical quantity of

water that is liberatable during esterification of the cyanohydrins. When the desiccant itself is not a solvent, an inert water-immiscible solvent such as a saturated hydrocarbon, e.g., hexane or heptane, a halogenated hydrocarbon, e.g., chloroform or carbon tetrachloride, or an ether, e.g., diethyl ether, is preferably employed as a means of facilitating temperature control.

The esterification reaction will normally be substantially complete after about  $\frac{1}{2}$  to about 6 hours, depending upon the reaction temperature and the strength of the nitrating agent. Excellent results have been obtained with approximately 98 percent nitric acid, a reaction temperature of about  $5^{\circ}$  to  $10^{\circ}$  C. and a reaction period of 2 to 3 hours.

When the reaction is substantially complete, the reaction mixture is quenched by dilution, preferably with water. Higher molecular weight cyanohydrin nitrates, that is, those having a water-insolubilizing hydrocarbon substituent containing 5 or more carbon atoms, will normally separate from the diluted reaction mixture of their own accord and can be recovered by decanting. Lower molecular weight cyanohydrin nitrates are miscible in substantial proportions with the dilute aqueous acid and are accordingly conveniently separated by the use of an inert, water-immiscible, organic selective solvent therefor, such as methylene chloride, chloroform, carbon tetrachloride, diethyl ether, or the like.

The preparation of the cyanohydrins from which the nitrates are derived is conventional, and as such, does not form the essence of this invention.

The aldehyde and ketone cyanohydrin nitrates whose use is included by this invention can be incorporated in the hydrocarbon fuel oils disclosed herein in any suitable manner. These materials are normally soluble in paraffinic as well as aromatic hydrocarbons in the proportions disclosed herein, and therefore can be incorporated directly in the fuel oils. Because of the small proportions in which the materials disclosed herein are used, it may be preferable from the standpoint of rapidly facilitating formation of a homogeneous mixture to employ such materials in the form of concentrated solutions of, say, 10 to 50 percent strength in a solvent that is compatible with the fuel oil.

#### Examples I and II

In order to determine the effectiveness of compounds of the class indicated herein, representative compounds of such class were prepared and incorporated in varying proportions in several base fuels having predetermined cetane numbers, and the thus obtained fuel compositions were tested to determine their cetane numbers as modified by the test compounds. The base fuels tested were as follows: Test fuel 1 was a commercial, straight run diesel fuel meeting the ASTM requirements for a grade 2-D or medium diesel fuel. Test fuel 2 consisted of a blend of 40 volume percent West Texas straight run No. 2 fuel oil distillate, 40 volume percent of a fluid catalytically

|    |                                                  | Test Fuel 1 | Test Fuel 2 |
|----|--------------------------------------------------|-------------|-------------|
| 5  | Gravity, ° API                                   | 38.9        | 32.0        |
|    | Viscosity, Kinematic, cs. (SUS) $100^{\circ}$ F. | 2.47        | 2.06 (32.8) |
|    | Flash Point, ASTM D-93, ° F.                     | 152         | 154         |
|    | Water and Sediment, Percent                      | —           | trace       |
|    | Carbon Residue, ASTM D-96, Percent               | —           | 0.031       |
|    | Sulfur, ASTM D-1266                              | 0.121       | 0.598       |
|    | Ash, Percent                                     | <0.01       | <0.01       |
| 10 | Distillation, Gas Oil:                           |             |             |
|    | Over Point, ° F.                                 | 346         | 332         |
|    | End Point, ° F.                                  | 634         | 596         |
|    | 10% Evap. at, ° F.                               | 423         | 411         |
|    | 90% Evap. at, ° F.                               | 574         | 546         |

15 The cyanohydrin nitrates tested were prepared by nitration of appropriate cyanohydrins. The cyanohydrins from which the cyanohydrin nitrates subjected to testing were derived comprised both a ketone cyanohydrin (acetone cyanohydrin) and an aldehyde cyanohydrin (2-ethylhexaldehyde cyanohydrin). The respective cyanohydrins were separately prepared by admixture of 0.6 mole of acetone and freshly distilled 2-ethylhexaldehyde, respectively, with separate mixtures of 1.0 mole of potassium cyanide in 250 milliliters of anhydrous ether. Acetic acid in the amount of 50 milliliters was added dropwise to each mixture with stirring over a 15-minute period. The temperatures of the reaction mixtures were held at  $15\text{--}20^{\circ}$  C. during such addition. The reaction mixtures were then stirred for 3.5 hours at  $20^{\circ}$  C. After standing overnight at room temperature, the solid (potassium acetate) was filtered off from each mixture and washed with two 50 milliliter portions of anhydrous ether. The solvent was then removed from the combined filtrate and washings. Yields approaching theoretical were obtained.

20 Acetone- and 2-ethylhexaldehyde-cyanohydrin nitrates were then prepared by nitration of the above-indicated cyanohydrins, using separate nitrating mixtures consisting of about 92.5 grams of white fuming nitric acid ( $d=1.49\text{--}1.50$ ) added to about 246 milliliters of acetic anhydride. External cooling was employed while mixing to maintain the temperature below  $35^{\circ}$  C. The nitrating mixtures were chilled to  $5^{\circ}$  C. and 0.6 mole of the respective cyanohydrins were added in one portion to the respective nitrating mixtures. The mixtures were stirred at  $8\text{--}10^{\circ}$  C. for 15 minutes and for 1.5 hours at room temperature. The reaction mixtures were then poured over separate 500 gram portions of crushed ice and stirred for one hour. Acetone-cyanohydrin nitrate was extracted 25 from the appropriate reaction mixture with three 150 milliliter portions of methylene chloride. The 2-ethylhexaldehyde-cyanohydrin nitrate separated spontaneously from the water-acetic acid solution. This product was water-washed, dried over anhydrous sodium sulfate and distilled at reduced pressure. The properties of the respective cyanohydrin nitrates, hereinafter referred to 30 respectively as test compounds A and B, were as follows:

|                                                           | Density, 25° C. | Yield, percent | B.P., ° C.          | $n_{D}^{20}$ | Nitrogen, percent |       |
|-----------------------------------------------------------|-----------------|----------------|---------------------|--------------|-------------------|-------|
|                                                           |                 |                |                     |              | Calculated        | Found |
| Acetone Cyanohydrin Nitrate (Test Compound A).            | 1.127           | 64.1           | 64-65 (10 mm. Hg.)  | 1.4180       | 21.53             | 20.91 |
| 2-Ethylhexaldehyde Cyanohydrin Nitrate (Test Compound B). | 1.017           | 72.5           | 77-79 (1.4 mm. Hg.) | 1.4419       | 14.00             | 13.76 |

cracked No. 2 fuel oil distillate, and 20 volume percent of a Thermophor catalytically cracked No. 2 fuel oil distillate, said blend being one meeting the ASTM requirements for a grade 2-D diesel fuel. Inspection data for the base fuels were as follows:

75 The test fuel oil compositions containing the cyanohydrin nitrates were tested for cetane number under standard test procedure ASTM D613-48T, described in the ASTM Manual of Engine Test Methods for Rating Fuels for 1952, at pages 63-71. Briefly, this test involves

comparing the ignition quality of an unknown test fuel under standard operating conditions with the ignition quality of reference fuel blends having known cetane numbers. The test is carried out in a single cylinder diesel engine having a continuously variable compression ratio. During the test the compression ratio is varied for the test fuel and the reference fuels to obtain a fixed "delay period," that is, the time interval between fuel injection and ignition. When the compression ratio that produces the fixed delay period for the test fuel has been determined to be between the compression ratios that will produce the same delay period for two reference fuel blends that differ by not more than 5 cetane numbers, the rating of the sample is calculated by interpolation. The standard reference fuels are prepared from n-cetane and  $\alpha$ -methylnaphthalene meeting ASTM standards. However, secondary, petroleum distillate reference fuels that have been calibrated against the standard blends are normally used for routine testing. The operating conditions of the test are as follows:

|                                    |                   |
|------------------------------------|-------------------|
| Engine speed, r.p.m.               | 900 $\pm$ 0       |
| Injection advance, deg. B.T.D.C.   | 13.0              |
| Injection opening pressure, p.s.i. | 1500 $\pm$ 50     |
| Injection quantity, ml./min.       | 13.0 $\pm$ 0.2    |
| Injector pintle valve lift, in.    | 0.005 $\pm$ 0.001 |
| Injector water jacket temp., ° F.  | 100 $\pm$ 5       |
| Valve clearances, hot, in.         | 0.008 $\pm$ 0.001 |
| Crankcase lubricating oil—         |                   |
| SAE grade                          | 30                |
| Viscosity, sec., SUV/130° F.       | 185-255           |
| Oil pressure, p.s.i.               | 25-30             |
| Oil temperature, ° F.              | 135 $\pm$ 15      |
| Coolant temperature, ° F.          | 212 $\pm$ 3       |
| Intake air temperature, ° F.       | 150 $\pm$ 1       |

The results of the foregoing tests are presented in the following table:

|                                          | 1    | 2    | 3    | 4    | 5    | 6    | 7    | 8    | 9    | 10   | 11   | 12   | 13   | 14   |
|------------------------------------------|------|------|------|------|------|------|------|------|------|------|------|------|------|------|
| Make-up:                                 |      |      |      |      |      |      |      |      |      |      |      |      |      |      |
| Base Fuel, Percent by Vol.—              |      |      |      |      |      |      |      |      |      |      |      |      |      |      |
| Test Fuel 1.....                         | 100  | 100  | 100  | 100  | 100  |      | 100  | 100  | 100  | 100  | 100  | 100  | 100  | 100  |
| Test Fuel 2.....                         |      |      |      |      |      | 100  |      |      |      |      |      |      |      |      |
| Addition Agent, Percent by Vol. (added)— |      |      |      |      |      |      |      |      |      |      |      |      |      |      |
| Test Compound A.....                     | 0.25 | 0.5  | 1.0  | 2.0  |      |      | 0.1  | 0.25 | 0.5  | 1.0  |      |      |      |      |
| Test Compound B.....                     |      |      |      |      |      |      |      |      |      |      | 0.25 | 0.5  | 1.0  |      |
| Inspection:                              |      |      |      |      |      |      |      |      |      |      |      |      |      |      |
| Cetane Number, ASTM D-613.....           | 54.0 | 61.8 | 63.4 | 63.6 | 64.5 | 35.8 | 37.7 | 40.0 | 43.5 | 45.8 | 52.4 | 55.3 | 57.9 | 63.2 |

From the data presented in the foregoing table it will be seen that both low and high cetane number fuels are improved by incorporation therein of compounds of the type whose use is included by the invention. The property demonstrated in the table appears to be shared by the other members of the class disclosed, although not necessarily equivalently. Therefore, it will be understood that the invention is not limited to the foregoing specific embodiments and that similar improvement in ignition quality can be obtained by admixture of the same or equivalent proportions of other cyanohydrin nitrates disclosed herein in the same fuel oils or in other hydrocarbon fuels disclosed herein. Examples of other fuel compositions of the preferred class are as follows:

|                                          | Example 3 | Example 4 | Example 5 | Example 6 | Example 7 | Example 8 |
|------------------------------------------|-----------|-----------|-----------|-----------|-----------|-----------|
| <b>Base Fuel:</b>                        |           |           |           |           |           |           |
| 1-D Diesel Fuel.....                     |           | x         | x         | x         |           | x         |
| 2-D Diesel Fuel.....                     | x         |           |           |           | x         |           |
| 4-D Diesel Fuel.....                     |           |           |           | x         |           |           |
| <b>Addition Agent, Percent by Wt.:</b>   |           |           |           |           |           |           |
| Acetaldehyde Cyanohydrin Nitrate.....    | 0.75      |           |           |           |           |           |
| Oxo-Octaldehyde Cyanohydrin Nitrate..... |           | 0.5       |           |           |           |           |
| Lauraldehyde Cyanohydrin Nitrate.....    |           |           | 0.5       |           |           |           |
| Dipropyl Ketone Cyanohydrin Nitrate..... |           |           |           | 1.0       |           |           |
| Butyrene Cyanohydrin Nitrate.....        |           |           |           |           | 0.75      |           |
| Laurone Cyanohydrin Nitrate.....         |           |           |           |           |           | 0.5       |

6  
Good ignition quality will also be obtained with the following fuel compositions which are examples of other compositions within the scope of this invention:

|                    | Addition Agent                                         | Wt. Proportion Addition Agent | Base Fuel            |
|--------------------|--------------------------------------------------------|-------------------------------|----------------------|
| 10 Example 9.....  | Stearaldehyde Cyanohydrin Nitrate.....                 | 1.0                           | 1-D Diesel Fuel..... |
| Example 10.....    | Benzaldehyde Cyanohydrin (Mandelonitrile) Nitrate..... | 1.0                           | Do.                  |
| Example 11.....    | p-Tolualdehyde Cyanohydrin Nitrate.....                | 1.0                           | Do.                  |
| 15 Example 12..... | 1-Naphthaldehyde Cyanohydrin Nitrate.....              | 1.0                           | Do.                  |
| Example 13.....    | Cinnamaldehyde Cyanohydrin Nitrate.....                | 1.0                           | Do.                  |
| Example 14.....    | Crotonaldehyde Cyanohydrin Nitrate.....                | 1.0                           | Do.                  |
| Example 15.....    | Anthraldehyde Cyanohydrin Nitrate.....                 | 1.0                           | Do.                  |
| 20 Example 16..... | Cyclohexaldehyde Cyanohydrin Nitrate.....              | 1.0                           | Do.                  |
| Example 17.....    | Cyclopentaldehyde Cyanohydrin Nitrate.....             | 1.0                           | Do.                  |
| Example 18.....    | Furfural Cyanohydrin Nitrate.....                      | 1.0                           | Do.                  |
| Example 19.....    | 2-Nonadecanone Cyanohydrin Nitrate.....                | 1.0                           | Do.                  |
| 25 Example 20..... | Acetophenone Cyanohydrin Nitrate.....                  | 1.0                           | Do.                  |
| Example 21.....    | 1-Isobutyronaphthone Cyanohydrin Nitrate.....          | 1.0                           | Do.                  |
| Example 22.....    | Benzophenone Cyanohydrin Nitrate.....                  | 1.0                           | Do.                  |
| Example 23.....    | Dicyclobutyl Ketone Cyanohydrin Nitrate.....           | 1.0                           | Do.                  |
| 30 Example 24..... | Cyclopentanone Cyanohydrin Nitrate.....                | 1.0                           | Do.                  |
| Example 25.....    | Cyclohexanone Cyanohydrin Nitrate.....                 | 1.0                           | Do.                  |
| Example 26.....    | 1-(2-furyl)-1-butane Cyanohydrin Nitrate.....          | 1.0                           | Do.                  |

It is emphasized that the presence of both a nitrate

ester group and a nitrile group is important for the purposes of this invention, as this combination results in superior ignition quality improvement. For example, test compounds A and B were compared for effectiveness as ignition quality promoters against amyl nitrate, a typical alcohol nitrate ignition quality promoter. In these tests test compound A, test compound B and amyl nitrate were incorporated in a diesel fuel having a cetane number of 50-55 clear, in the proportion of 0.5 percent by volume each, which corresponded respectively to proportions of 0.00433, 0.00237 and 0.00373 mol per 100 g. of oil, and the resulting cetane number improvement determined by the procedure of ASTM D613-48T, described elsewhere

50

55

60

herein. The respective cetane number improvements, corrected to 0.00237 mol/100 g. fuel, were as follows:

|                             | Test Compound A | Test Compound B | Amyl Nitrate |
|-----------------------------|-----------------|-----------------|--------------|
| Cetane Number Increase..... | 5.1             | 5.5             | 4.1          |

From a comparison of the foregoing figures it will be seen that when both a nitrile and a nitrate group are attached to the same carbon atom, superior results are obtained.

ASTM grade 1-D, 2-D and 4-D diesel fuels are defined in ASTM Standards on Petroleum Products and Lubricants, November 1956, under ASTM designation D975-53T. Number 2 fuel oils are defined in the same reference under ASTM designation D396-48T.

The hydrocarbon fuel oil compositions of this invention may contain in addition to the cyanohydrin nitrates disclosed herein other addition agents adapted to improve the oils in one or more respects. For example, the fuel oil compositions of this invention may also contain oxidation inhibitors, corrosion inhibitors, detergents, sludge inhibitors, anti-foam agents and other ignition quality or combustion improvement agents.

It will be apparent to those skilled in the art that many modifications and variations of the invention as described herein can be made without departing from the spirit or scope thereof. Accordingly, only such limitations should be imposed as are indicated in the claims appended hereto.

I claim:

1. A fuel oil composition comprising a major amount of a hydrocarbon fuel oil and containing a small amount, sufficient to improve the ignition quality of said oil, of a cyanohydrin nitrate derived from a member of the group consisting of aldehydes and ketones having as one

substituent a hydrocarbon radical containing 1 to 18 carbon atoms and as the other a member selected from the group consisting of a hydrocarbon radical of the same kind and hydrogen.

5. 2. The composition of claim 1 where the small amount is about 0.05 to 2 percent by weight of the composition.
3. The composition of claim 1 where the hydrocarbon radical is an alkyl group that contains 1 to 12 carbon atoms.
10. 4. A fuel oil composition comprising a major amount of a diesel fuel and a small amount, sufficient to improve the ignition quality of said oil, of acetone cyanohydrin nitrate.
15. 5. The composition of claim 4, where said small amount is about 0.5 to 1 percent by weight of the composition.
20. 6. A fuel oil composition comprising a major amount of a diesel fuel and a small amount, sufficient to improve the ignition quality of said oil, of 2-ethylhexaldehyde cyanohydrin nitrate.
25. 7. The composition of claim 6, where said small amount is about 0.5 to 2 percent by weight of the composition.

25. References Cited in the file of this patent

UNITED STATES PATENTS

- |              |                 |               |
|--------------|-----------------|---------------|
| 2,066,506    | Woodbury et al. | Jan. 5, 1937  |
| 2,274,629    | Ellis           | Feb. 24, 1942 |
| 30 2,392,610 | Noland et al.   | Jan. 8, 1946  |
| 2,392,611    | Nygaard et al.  | Jan. 8, 1946  |
| 2,438,452    | Pollock         | Mar. 23, 1948 |

OTHER REFERENCES

35. "Means of Improving Ignition Quality of Diesel Fuels," by Nygaard et al., "Journal of the Institute of Petroleum Technology," vol. 27, pp. 348-368, October 1941.